

## UNITED STATES PATENT OFFICE

2,538,751

## INKING ROLLER MANUFACTURE

Edward D. Hill, Cleveland, Ohio

No Drawing. Application April 1, 1948,  
Serial No. 18,490

6 Claims. (Cl. 117—46)

1

Inking rollers as used in printing and graining have long been made of glue modified by glycerin or molasses or the like-acting agent, and such glue-base body has been regarded as very satisfactory with respect to its resiliency and follow-up. The rather soft gel consistency of the glue body provides enough give and resilience to satisfactorily operate on type and plate surfaces, even though of considerable irregularity and complexity. However, the glue-base roller has the very serious drawbacks of being highly susceptible to atmospheric changes, and to the action of drying oils and solvents common in ink compositions. Various substitutes have been proposed from time to time, and particularly rubber and vulcanized oil compositions have been tried, but these have had the objection of being too different in their body consistency to give general satisfaction, and besides, such materials are susceptible to the action of oils and solvents in inks.

By the present invention, it now becomes possible to realize the excellent body properties of the glue-base material, and at the same time obviate its disadvantages above-indicated. Thus, an ink carrier or roller may be had with the resilience and body characteristics of glue-base material but with immunity to change from atmospheric variations and with resistance against detrimental action of ink oils and solvents. Other objects and advantages of the invention will appear from the following description.

To the accomplishment of the foregoing and related ends, the invention, then, comprises the features hereinafter fully described and particularly pointed out in the claims, the following description setting forth in detail certain illustrative embodiments of the invention, these being indicative, however, of but a few of the various ways in which the principle of the invention may be employed.

A glue-base material is made up into roller form, or in fact any glue-base roller may be taken as the starting point for the present invention. As well-known, a common composition is glue about one part and glycerin or molasses about three parts, and such composition, liquefied on a water bath and brought to uniformity, is cast in roller form on a metal mandrel or shaft. Such a roller is here finished by providing a surface or outside layer having unique properties. For this, a synthetic resin reaction product of olefinic halides and alkali sulphide, generally known as polyalkylene or a polysulphide synthetic resin is made up with a plasticizer or extender, and an agent reactive on the synthetic resin and on glue.

5 The polysulphide resins are described in chemical literature, and for instance in Fieser's "Organic Chemistry" (pub. by D. C. Heath & Co., Boston, 1944), page 342, and a commercially available resin of this order sold under the name "Thiokol" is satisfactory for the purpose. The extender is a high boiling miscible agent which is liquid at temperatures between about 100 and 212° F., and a phthalate ester, e. g. dibutyl phthalate is illustrative. Other esters or phthalates or other agents with like properties may be employed, e. g. dioctyl phthalate, dihexyl phthalate, tri-cresyl phosphate, etc. The amount of the phthalate or the like may be about 10-35 per cent, and usually about 25 per cent by weight. The proportioning is in general such as to give a modified resin with similar body properties as the glue base. This makes possible the temporary deformation of the glue-base roller in service without 10 disruption of the thin resin facing which is applied. With the resin mixture as just noted, there is incorporated also an agent reactive on both the resin and the glue. This toughens or cures the resin and bonds it mutually with the 15 glue roller to which it is applied as a facing. The reactive agent may be an aldehyde, preferably furfural, although others which are miscible, as benzaldehyde, hexamethylenetetramine, etc. may be employed. The amount of the furfural or the like is in general about 10-32 per cent, and desirably around 20 per cent. If too small an amount 20 is employed, the resin is not sufficiently toughened or is lacking in desired resistance. If too much is employed, the material tends to be lacking in 25 desired elasticity. With the aldehyde or the like an acid reaction or medium is supplied, and this requires a weak or dilute acid. Desirably, formic acid in amount of 5 to 15 per cent is satisfactory, preferably 10 per cent based on the amount of 30 the aldehyde. Correspondingly, other acids which are miscible, as salicylic acid, furoic acid, etc. may be used. It is noticed, as a particular feature here, that the synthetic resin which is to form the 35 actual surface of the roller, enclosing the glue body, as a polysulphide contains sulphur, which is also reactive on glue, and in addition, it is provided with furfural or the like which is again reactive upon the resin and the glue. Thus, when the resin composition is brought into contact with 40 the glue surface, under proper conditions, there is sufficient interaction to bond the resin substantially integrally to the glue-base body. While the synthetic resin as a sheet, or preferably a thin film, may in some cases be assembled with the 45 glue-base body, as by casting the latter there-

2

against, it is better in practice to apply the synthetic resin as a liquid to the pre-formed glue-base body. For this, the polysulphide resin composition including the furfural or the like and weak acid, is brought to uniform liquid condition at a temperature within the range of 100° to about 200° F., and desirably, for instance, at around 160° F., and the material is applied to the glue-base roller in any convenient manner, depending upon the size of the roller, etc. And the present composition may be applied by, for instance, a traveling spout or feeder on the roller as rotated, or the roller may be rotated in partial immersion or may be dipped; and a final rotation apart from the applicator serves to distribute the material in a uniform film coat. Preferably, the resin surfacing may be quite thin, for instance 0.001-0.005 in., although of course in conditions where a thick surface of the resin is desired, a thicker layer may be employed. In general, the control of the thickness of such applied material may be controlled as desired by variation in the amount of the phthalate or other extender, and also by variation in the temperature at which the resin composition is applied. Where desired, the freshly coated surface may have a gas flame passed over it. This flash heating thus momentarily applied accelerates the curing and insures smoothness. The resin surface cools and sets quickly, and the aldehyde or curing agent toughens it thence at ordinary temperature, so that such rollers may be ready for use in twenty-four hours.

An important feature of the present construction is the action of an agent in common on both the synthetic resin layer and the glue-base body. Instead of separable resin and glue body, the construction provides a substantially integral material, body and surface, and the surface layer cannot be stripped from the body. If tearing be induced, the rupture goes in the glue body instead of between the synthetic resin surface and the glue. It is thus seen that such roller construction, with its glue-base body, preserves all of the desirable resilience and softness of the conventional glue-base roller, but now guarded and sealed over against detriment from atmospheric change and ink-ingredients. Such facing on the roller is sufficiently uniform with the body properties of the roller to maintain the true glue body characteristics, but the synthetic resin surface is impervious to atmospheric moisture and is also resistant to the other ingredients common in printing and graining inks which cause cracking and damage to glue rollers. Furthermore, this synthetic resin surface takes and carries inks with the same efficiency as a glue-base surface, but at the same time it very substantially excels a glue-base surface in its resistance to wear. Such an inking roller thus has a service life materially greater than obtainable with the customary rollers.

Other modes of applying the principle of the invention may be employed, change being made as regards the detail described, provided the features stated in any of the following claims, or the equivalent of such, be employed.

I therefore particularly point out and distinctly claim as my invention:

1. The method of forming an inking roller which comprises mixing a polyalkylene polysulphide synthetic resin with an extender selected

from the group consisting of dibutyl phthalate, dioctyl phthalate, dihexyl phthalate and tricresyl phosphate; a miscible aldehyde reactive with the resin; and a weak acid selected from the group consisting of formic acid, salicylic acid, and furoic acid; the aldehyde being present in the amount of between about 10% and about 32%, liquefying the mixture by warming the same to a temperature within the range of about 100° F. to about 200° F., applying a layer of such liquid mixture to a glue-base roller, and finally curing the resin and bonding the same to said glue base roller.

2. The method of forming an inking roller which comprises mixing a polyalkylene polysulphide synthetic resin with an extender selected from the group consisting of dibutyl phthalate, dioctyl phthalate, dihexyl phthalate and tricresyl phosphate; furfural; and a weak acid selected from the group consisting of formic acid, salicylic acid, and furoic acid; the furfural being present in the amount of between about 10% and about 32%, liquefying the mixture by warming the same to a temperature within the range of about 100° F. to about 200° F., applying a layer of such liquid mixture to a glue-base roller, and finally curing the resin and bonding the same to said glue-base roller.

3. The method of forming an inking roller which comprises mixing a polyalkylene polysulphide synthetic resin with an extender selected from the group consisting of dibutyl phthalate, dioctyl phthalate, dihexyl phthalate and tricresyl phosphate; a miscible aldehyde reactive with the resin; and a weak acid selected from the group consisting of formic acid, salicylic acid, and furoic acid; the aldehyde being present in the amount of between about 10% and about 32%, liquefying the mixture by warming the same to a temperature within the range of about 100° F. to about 200° F., applying a layer of such liquid mixture to a glue-base roller, and finally surface-fusing and evening the synthetic resin by rapidly passing a flame thereover.

4. A glue-base roller surfaced with a polyalkylene polysulphide synthetic resin layer formed by the process of claim 1.

5. A glue-base roller surfaced with a polyalkylene polysulphide synthetic resin layer formed by the process of claim 2.

6. A glue-base roller surfaced with a polyalkylene polysulphide synthetic resin layer formed by the process of claim 3.

EDWARD D. HILL.

#### REFERENCES CITED

The following references are of record in the file of this patent:

#### UNITED STATES PATENTS

| Number       | Name          | Date           |
|--------------|---------------|----------------|
| 294,436      | Bingham       | Mar. 4, 1884   |
| 1,098,776    | Arsen         | June 2, 1914   |
| 1,239,630    | Soane         | Sept. 11, 1917 |
| 65 1,846,810 | Lewis et al.  | Feb. 23, 1932  |
| 1,963,856    | Lewis et al.  | June 19, 1934  |
| 2,195,380    | Patrick       | Mar. 26, 1940  |
| 2,204,383    | Safford       | June 11, 1940  |
| 2,271,124    | Juve et al.   | Jan. 27, 1942  |
| 70 2,304,001 | Kugler et al. | Dec. 1, 1942   |
| 2,453,735    | Toland et al. | Nov. 16, 1948  |